

(Model.)

G. F. WILSON & P. O'REILLY.  
Preparation of Paper Stock from Colored Rags.

No. 227,463.

Patented May 11, 1880.



WITNESSES.

Philip Maney  
C. J. Hedrick

INVENTORS.

George F. Wilson and  
Philip O'Reilly by  
A. F. O'FolliR their atty.

# UNITED STATES PATENT OFFICE.

GEORGE F. WILSON, OF EAST PROVIDENCE, AND PHILIP O'REILLY, OF PROVIDENCE, RHODE ISLAND.

## PREPARATION OF PAPER-STOCK FROM COLORED RAGS.

SPECIFICATION forming part of Letters Patent No. 227,463, dated May 11, 1880.

Application filed April 12, 1880. (Specimens.)

To all whom it may concern:

Be it known that we, GEO. F. WILSON, of East Providence, and PHILIP O'REILLY, of Providence, both of the State of Rhode Island, 5 have invented a new and useful Improvement in Preparation of Paper-Stock from Colored Rags, which improvement is fully set forth in the following specification.

The object of our invention is to discharge 10 the coloring-matter from old or new rags or cloth and other kinds of paper-stock, and to render the same white without injury, or comparatively so, to the texture or to the fiber of the material.

15 So far as we are aware the course practically pursued by paper manufacturers in preparing their paper-stock for use is as follows:

The stock is put into the well-known form 20 of apparatus and boiled for several hours in a solution of quicklime, or of soda-ash, or caustic soda and quicklime, for the double purpose of removing the oils or greasy matters adherent to the stock and for discharging 25 the colors. It often happens that the greasy matters are rendered insoluble, or the coloring-matters are rendered more prominent, so as seriously to interfere with the action of the chloride of lime, to which the stock is subsequently subjected for bleaching 30 purposes.

In discharging colors from misprints or calicoes the mordants are usually removed by various acid baths adapted to the particular mordants; after which the colors can be easily 35 removed by alkalies. This process, however, affects more or less injuriously the strength of the cloths.

We have found that the mordants can be 40 treated with chemicals in such a manner that a double decomposition in the bath will take place in contact with the colors, and the effect of this nascent action, so produced, will be to produce the oxidation or deoxidation 45 of the mordants, and that the discharge of the coloring-matters may be brought about without injury to the fabrics or paper-stock so treated.

In order to enable those skilled in the art

to carry into effect our invention, we will describe our process and the chemicals we prefer to use in it, reference being had to the annexed drawing, which forms a part of this specification.

In said drawing is shown an apparatus which we have devised to save labor and to utilize 55 to the utmost extent all of the chemicals employed.

A represents an iron-wire basket with a strong iron frame, which holds the paper-stock in the several processes until it is bleached and 60 ready to be dried. This basket is suspended by a rope passing over a pulley, so that it can be readily raised and lowered. This pulley is suspended from a carrier, B, which travels on a rail, C. Beneath this rail, and in a line 65 with its length, is a series of keirs, D E F G H. The basket A can, by raising and lowering it and moving the carrier B, be readily transferred to any of the keirs.

In connection with the keir H a stirring device, I, is employed. This is so constructed as to be raised and lowered. It is supported in a bearing attached to the bar or rail K, so as to be revolved by means of the belt or strap on the pulley L. The spindle or arbor of the 75 stirrer passes through the hub of the pulley, and is free to move up and down therein and in its bearing; but rotary movement independent of the pulley is prevented by a spline-and-groove connection.

From the upper part of the spindle of the stirrer a rope passes over a pulley, M, so that the stirrer may be raised, as shown in full lines, or lowered into the keir, as shown in dotted lines, as required.

A cover is or may be employed for the keir H. It is made to serve as a step or bearing for the spindle of the stirrer, as well as to close the keir.

The operation of preparing or bleaching the 90 stock is as follows: The first step is to put in the wire basket a suitable quantity—say five hundred pounds—of colored rags cut into small pieces, as is the common practice, for convenience in working them. Into the keir 95 D are put, for treating the weight of rags men-

tioned, five hundred gallons of water and fifteen pounds of caustic soda, to which is added a small quantity—say two gallons—of soft soap. We now put the wire basket and rags into the keir and boil them, preferably under atmospheric pressure, for about three hours, or sufficiently long to remove the oils and grease, which may be accomplished with frequent stirring in much less time. They may now be transferred in the basket to keir H, to be thoroughly washed with water. In washing the stirring apparatus is employed, it being let down into the position indicated in dotted lines in the drawing. The operation is continued until the stock is sufficiently clean, which an expert paper-maker will readily determine. The keir E is now supplied with two hundred and fifty gallons of water, with which has been mixed five pounds of a soluble salt of manganese, prepared for the purpose from black oxide of manganese and muriatic and sulphuric acids, as hereinafter described. The rags having been washed are now immersed in this solution, where they are to remain for about three hours, being thoroughly agitated or stirred during this whole or a portion of the time. While this process is going on we put into the keir F two hundred gallons of water having in solution fifteen pounds of chloride of lime, where the rags are thoroughly stirred and where they remain for about two hours. If the goods have obtained or taken on a brown color they may be washed thoroughly in the keir H, and then removed to the keir G, in which has been put two hundred and fifty gallons of water and five pounds of oxalic acid. This is for the purpose of removing any traces of iron or manganese which may be left in the rags. They are allowed to remain in this solution for about three hours, when they may be again washed in keir H, and then thrown into a hydro-extractor of any ordinary or suitable construction, which will take out nearly all the water remaining in them; after which they may be dried and made ready for shipment. The rags coming out of this process are ready to be beaten into pulp in the ordinary beating-engines.

Should the rags not have obtained the brown color referred to above they may be returned to the manganese solution again, and then again to the chloride-of-lime solution, as before. The remaining part of the processes following this second treatment will be the same as before described.

Permanganate of potash could be employed for the manganese with excellent results. We would prefer to use it but for economical reasons.

We have obtained nearly or quite as good results by means of the soluble salt of manganese, before referred to, which is prepared in the following way: In a suitable vessel, to one pound of black oxide of manganese we add one pound of commercial muriatic acid,

or other quantities in approximately the same proportion are used. We mix them well and let the whole remain for from thirty minutes to one hour, and then add two and one-half pounds of commercial sulphuric acid; stir and heat the mass gently until the manganese is dissolved, then we add about three gallons of water, stir it well, and leave the whole to settle. In charging the keir E only the clear liquor of the soluble salt of manganese is used.

We have indicated the proportions in the foregoing process with considerable minuteness in order that the invention could be readily carried into effect; but it is obvious that these may be varied more or less; and we do not conform ourselves strictly thereto. The stirring apparatus can, if desired, be readily constructed so as to be shifted from one keir to the other by supporting the bearing for the spindle of the stirrer in a traveling bracket, and making the elevating and lowering pulley also movable, like that which supports the basket. This is not, however, considered necessary, as the stirring is principally required in the washing-kier.

Having thus fully described our said invention, and the manner in which the same is or may be carried into effect, what we claim, and desire to secure by Letters Patent, is—

1. The method of discharging the color from colored rags or paper-stock by effecting a double decomposition in contact with the colors, so as to cause the oxidation or deoxidation of the mordants, and subsequently treating the stock with chloride of lime, substantially as described.

2. In discharging the color from paper-stock, the method of effecting a double decomposition in contact with the colors, by treating the rags or other stock, after removal of oils and grease, with soluble salt of manganese, permanganate of potash, or similar manganese compound, substantially as described.

3. In the preparation of colored rags or similar stock for paper-pulp, as described, the method of removing traces of iron or manganese by means of oxalic acid, substantially as described.

4. The process of preparing colored rags or similar stock for paper-pulp by boiling the stock with alkali to remove oils and grease, washing, treating it with a salt or other suitable compound of manganese, and then with chloride of lime, washing, and subjecting it to the action of oxalic acid, substantially as described.

5. The method of preparing a soluble manganese-salt for use, as hereinbefore set forth, by treating black oxide of manganese with muriatic and sulphuric acids, substantially as described.

6. The apparatus described, consisting of the series of keirs, the basket, means, substantially as indicated, for transferring said

basket, as required, from keir to keir, and a stirring device adapted to be raised and lowered, all essentially as set forth.

7. The combination of the stirrer, the bearing for its spindle or shaft, a pulley or gear connected therewith, as described, and means, as indicated, for raising and lowering the stirrer, substantially as set forth.

In testimony whereof we have signed this specification in the presence of two subscribing witnesses.

GEO. F. WILSON.  
PHILIP O'REILLY.

Witnesses:

CHARLES GREENE,  
AUGUSTUS S. MILLER.